

# United States Patent [19]

Webb

[11] 3,801,378

[45] Apr. 2, 1974

[54] NIOBIUM-GALLIUM SUPERCONDUCTOR

[75] Inventor: **George Wendell Webb, Princeton, N.J.**

[73] Assignee: **RCA Corporation, New York, N.Y.**

[22] Filed: Feb. 7, 1972

[21] Appl. No.: 224,000

[52] U.S. Cl..... 148/3, 75/174, 148/32,  
148/133, 325/216

[51] Int. Cl. .... C22c 27/00 H01f 1/01

[58] **Field of Search** ..... 148/2, 3, 11.5, 32, 32.5,  
148/133; 29/599; 75/174; 335/216

## [56] References Cited

UNITED STATES PATENTS

3,243,871 4/1966 Sauer

3,243,871 4/1966 Saur ..... 29/599  
3,256,118 6/1966 Speidel ..... 148/2

#### OTHER PUBLICATIONS

Naturwissenschaften, Vol. 54, No. 18, 1967 pp. 489 &

490.

Zeitschrift für Physik, 189, 1966, pages 401, 402 & 408-410.

Superconductors, Tanenbaum et al, New York, N.Y., 1962, Interscience Publishers, pages 42-45

Russian Journal of Inorganic Chemistry Vol. 9, No. 9,  
Sept. 1964 pgs 1172-1174.

*Primary Examiner*—Charles N. Lovell

*Attorney, Agent, or Firm*—Glenn H. Bruestle; Birgit E. Morris

[57]

## ABSTRACT

A superconducting alloy having a  $T_c$  of  $\geq 20\text{K}$  consists of a  $\beta$ -W alloy of Nb and Ga having the molar formula  $\text{Nb}_3\text{Ga}$ . The alloy can be formed by annealing a  $\beta$ -W phase Nb-Ga alloy at  $700^\circ\text{C}$ .

## 4 Claims, 5 Drawing Figures

PATENTED APR 2 1974

3,801,378

SHEET 1 OF 3



FIG. 1.

Fig. 2.Fig. 3.Fig. 4.



Fig. 5.

## NIOBium-GALLIUM SUPERCONDUCTOR

## BACKGROUND OF THE INVENTION

This invention relates to superconducting alloys and particularly to superconducting alloys of niobium and gallium.

Superconductivity in beta-tungsten ( $\beta$ -W) compounds of niobium and gallium was reported in 1958 by E. A. Wood et al., in *Acta Crystallogr.* 11, 604 (1958). The critical temperature ( $T_c$ ) of that compound, i.e., the temperature at which the onset of superconductivity was observed, was reported as being 14.5°K. G. Meyer reported in *Naturweiss* 18, 489 (1967), resistive transition onset of 19.85°K for a Nb-Ga alloy comprising nominally 15 atomic percent Ga. This alloy, however, had a transition width of 5°K and only a small percentage of the sample was superconducting at 19.0°K. While this material may possibly have contained the alloy identified and claimed by the applicant herein, there is no way to know this as no separate phase as claimed herein was identified by Meyer.

In addition to the above, G. Otto reported transitions of 16°K for Nb-Ga alloys having a nominal composition comprising 25 atomic percent Ga.

I have discovered a Nb-Ga alloy having a  $\beta$ -W structure and comprising about 25 atomic percent Ga which has a superconductivity onset as high as 20.3°K and having transition widths as low as 0.7°K. This alloy is not stable above about 700°C. It is this fact that probably accounts for the failure of others to observe this alloy in the past and which adds import to its method of preparation. The superconducting transitions reported by me were measured by the well-known inductive method.

## SUMMARY OF THE INVENTION

A superconducting alloy of Nb and Ga is characterized in that it has a  $\beta$ -tungsten structure, and a molar formula  $Nb_3Ga$ .

The novel superconducting alloy referred to above is prepared by annealing a  $\beta$ -tungsten-containing alloy of Nb-Ga at a temperature no greater than about 700°C.

## BRIEF DESCRIPTION OF THE DRAWINGS

FIG. 1 is a photomicrograph of a multiphase alloy of Nb-Ga exhibiting both a  $\beta$ -W phase and a  $Nb_5Ga_3$  phase.

FIG. 2 is a plot of  $T_c$  onset as a function of the  $\beta$ -W lattice constant for specimens with well defined onsets and sharp X-ray diffraction patterns.

FIG. 3 is a graph showing the superconducting onset of a Nb-Ga sample comprising a  $Nb_3Ga$  phase.

FIG. 4 is a graph showing the critical magnetic field as a function of temperature for  $Nb_3Ga$ ,  $Nb_3Sn$  and  $Nb_3Al$ .

FIG. 5 gives the relevant portion of the Nb-Ga phase diagram and the  $T_c$  as a function of the temperature of the final anneal.

## DETAILED DESCRIPTION OF THE INVENTION

The novel superconducting alloy is a  $\beta$ -W alloy and contains about 25 atomic percent Ga. It may be represented by the formula  $Nb_3Ga$ . The novel Nb-Ga alloys may include other phases together with the  $Nb_3Ga$  and, in fact, usually do. For example, FIG. 1 is a photomi-

crograph of a Nb-Ga alloy at 1,000 x magnification. The nominal composition of the alloy is 32 atomic percent Ga and 68 atomic percent Nb. The specimen was formed by quenching the alloy from the melt at 1,850°C to room temperature and subsequently annealing the quenched material for 47 hours at 700°C. The resultant superconducting material was determined to consist of two phases, one phase, i.e., the  $\beta$ -W phase, is the dark dendritic structure on the photomicrograph and has an average width of 1.5 $\mu$ . This phase has the molar formula  $Nb_3Ga$  and is characterized by the lattice parameter,  $a_0$ , of from 5.163 – 5.167. The remainder of the sample is  $Nb_5Ga_3$ . This sample had a superconductive onset  $T_c$  of 20.3°K.

15 The  $Nb_3Ga$   $\beta$ -W phase of the novel superconducting alloys typically have a lattice constant of from about 5.163 to 5.168. The lower the lattice constant, generally, the higher the measured value of  $T_c$ .

20 FIG. 2 is a plot of  $T_c$  onset as a function of  $\beta$ -W lattice constant for specimens with both well defined onsets and sharp x-ray diffraction patterns. Error bars indicate the range of lattice constants present in a given specimen as determined from the [622] X-ray diffraction line. Errors in the value of the mean of the lattice

25 constant are estimated to be  $\pm 0.001 \text{ \AA}$ . These latter errors are not shown in the plot. Points marked 0 are arc-melted specimens; those marked x are vapor deposited specimens and  $\Delta$  and  $\square$  are values of specimens as recited in Wood et al., supra, and G. F. Otto, *Z. fur Physik* 215, 323 (1968). It can readily be seen from the plot that the lattice constant of the specimen is critical to a high  $T_c$ . Generally, only specimens having a  $\beta$ -W phase with a mean value of  $a$  of less than about 5.168 exhibit values of  $T_c$  of  $\geq 20.0^\circ\text{K}$ .

35 The typical narrow width of the superconductive onset of the novel alloys can be seen with reference to FIG. 3 showing the change in inductance as a function of temperature.

40 The novel superconductor,  $Nb_3Ga$ , with a mean lattice constant of  $\leq 5.168$  is superior to other binary superconductor materials not only in the fact that it can be made to have a higher  $T_c$  than prior art binary superconductors, but also in the fact that higher magnetic fields can be applied to the novel superconductor. A comparison of the critical magnetic fields ( $H_{c2}$ ) in kilogauss as a function of temperature in °K for  $Nb_3Ga$ ,  $Nb_3Sn$  and  $Nb_3Al$  may be seen with reference to FIG. 4. It is apparent from the figure that  $Nb_3Ga$  has a considerably higher  $H_c$  than these other binary alloys of niobium.

45 The fact that Nb-Ga alloys having a  $\beta$ -W phase of the composition  $Nb_3Ga$  and a lattice constant of 5.163 – 5.168 has not been found heretofore is probably due to the instability of this phase at temperatures above about 700°C. In fact, this phase is formed by prolonged annealing of Nb-Ga alloys at 700°C. It may also be formed by vapor phase deposition at 700°C, however, the lattice constants of vapor phase grown specimens have not, to date, been as low as are grown and then annealed specimens. The vapor deposited specimens generally have values of  $T_c$  below that of arc grown material, i.e.,  $T_c$  of about 19°K. These materials are nevertheless potentially more useful than  $Nb_3Sn$  because of their high  $H_{c2}$ .

50 55 60 65 The complexity of the Nb-Ga alloy system can be seen with relation to the phase diagram of FIG. 5. It is apparent that a pure  $\beta$ -W phase cannot be formed in

a Nb-Ga alloy system when the specimen is prepared from the melt. When preparing the novel alloy from the melt, it is preferred to use a nominal composition of from about 20 to 33 atomic percent gallium and 67 - 80 atomic percent niobium. The pure materials are typically melted at a temperature of about 1,850°C and the melt is quenched. The alloy thus formed is then annealed at 700°C for extended periods of, for example, from 8 hours to several days. It can be seen from FIG. 5 that annealing at temperatures of about 700°C is important in obtaining high  $T_c$  specimens. The characteristics of several specimens prepared from different nominal atomic percentages of gallium and heat treated under different conditions is given in Table 1.

It can be seen from the table below that only those specimens which were annealed at 700°C or below (660°C) exhibited a  $T_c$  onset of  $\geq 20^\circ\text{K}$ . The specimens which were not annealed and the specimen an-

nium and gallium comprising a  $\beta$ -tungsten phase characterized by a mean lattice constant of from 5.163 to 5.168 comprising the steps of:

- 5 a. forming a melt of gallium and niobium, said melt consisting of from 20 to 33 atomic percent of gallium and from 67 to 80 atomic percent of niobium;
- b. quenching said melt to form a solid; and
- c. annealing said solid at a temperature of from about 600°C to about 700°C for extended periods of time to form the desired  $\beta$ -tungsten phase alloy.
- 10 2. A superconducting alloy having a  $T_c$  onset of  $\geq 20^\circ\text{K}$  comprising a  $\beta$ -tungsten phase having the molar formula  $\text{Nb}_3\text{Ga}$  and said alloy having an average lattice constant of from 5.163 to 5.168.
- 15 3. The superconducting alloy recited in claim 2 wherein said alloy has a  $T_c$  onset of at least 20.3°K.
4. The superconducting alloy recited in claim 2

TABLE 1

| Nominal<br>Ga<br>Comp | High Temp.<br>Heat<br>Treatment | Low Temp.<br>Anneal        | Inductance Change During<br>Transition |      |      | $\beta\text{-Wa}_0$<br>( $\text{\AA}$ ) | $a$         | $\text{Nb}_3\text{Ga}_3$<br>( $\text{\AA}$ ) | $c$   | X-Nb    |
|-----------------------|---------------------------------|----------------------------|----------------------------------------|------|------|-----------------------------------------|-------------|----------------------------------------------|-------|---------|
|                       |                                 |                            | onset<br>( $\text{K}^\circ$ )          | 20%  | 50%  |                                         |             |                                              |       |         |
| 21.5%                 | 1870°C                          | 163 hrs 660°C              | 20.1                                   | 19.9 | 19.8 | 19.7                                    | 5.163-5.178 | weak                                         | -     | present |
| 21.5%                 | 1870°C<br>powdered +            | 42 hrs 700°C               | 20.15                                  | 19.8 | 19.4 | 14.7                                    | 5.163-5.181 | weak                                         | -     | present |
| 24%                   | 1790°C                          | powdered +<br>23 hrs 700°C | 20.3                                   | 18.1 | 15.9 | 15.6                                    | 5.166-5.176 | weak                                         | -     | absent  |
| 32%                   | as arc<br>melted                | none                       | 16.5                                   | 14.8 | 14.6 | 13.9                                    | -           | -                                            | -     | absent  |
| 32%                   | 1850°C                          | none                       | 17.5                                   | 17.3 | 17.0 | 14.0                                    | 5.168-5.177 | 10.312                                       | 5.067 | absent  |
| 32%                   | 1850°C                          | 16 hrs 700°C               | 20.0                                   | 19.7 | 18.4 | 15.5                                    | 5.169-5.176 | 10.306                                       | 5.066 | absent  |
| 32%                   | 1850°C                          | 31 hrs 700°C               | 20.3                                   | 20.1 | 19.8 | 16.5                                    | 5.164-5.168 | 10.312                                       | 5.068 | absent  |
| 32%                   | 1850°C                          | 47 hrs 700°C               | 20.3                                   | 20.0 | 19.6 | 15.9                                    | 5.163-5.167 | 10.307                                       | 5.067 | absent  |
| 32%                   | 1850°C                          | 62 hrs 950°C               | 15.9                                   | 13.4 | 12.6 | 11.0                                    | 5.172-5.179 | 10.310                                       | 5.065 | absent  |
| 37%                   | as arc<br>melted                | none                       | $\geq 6$                               | -    | -    | -                                       | absent      | 10.306                                       | 5.066 | absent  |

nealed at 950°C all had critical temperatures significantly less than 20°K.

What is claimed is:

1. A method for preparing a superconducting alloy of

wherein the midpoint of transition is not less than 19.6°K.

\* \* \* \* \*